

## UNITED STATES PATENT OFFICE

1,954,922

METHOD FOR THE ALUMINOTHERMIC  
PREPARATION OF AIR QUENCHING STEEL

Clarence Leon Delachaux, Gennevilliers, France

No Drawing. Application January 22, 1932, Serial  
No. 588,242. In France January 6, 1930

5 Claims. (Cl. 75—45)

My invention is a continuation in part of my copending application Ser. No. 460,100.

My invention has for its object improvements in or relating to the aluminothermic self-hardening preparation of a self hardening steel adapted for welding purposes and containing beyond the usual components of mild steel, components such as nickel, chromium, molybdenum, tungsten and if required titanium, vanadium, boron and copper per.

It is known that in the case of the usual aluminothermic method of preparing steel, where the reaction  $Al + Fe_3O_4$  is executed at a high temperature about  $2500^{\circ} C.$  and ends very speedily, soft steel scrap is generally added to the aluminothermic mixture, said scrap serving to cool the reaction and being melted in its turn by the heat evolved by the aluminothermic reaction.

For obtaining certain alloy steels containing silicon and manganese, it has been already proposed to add instead of steel scrap an alloy containing manganese and silicon, said alloy being constituted for instance by grains.

This addition has a double part to play. On one hand the manganese and the silicon thus added act as deoxidizing or reducing agents. On the other hand part of this manganese and silicon remains in the final steel obtained.

In the case of my invention no manganese or silicon additions are provided with a view to increasing the contents of manganese or silicon in the final product, i. e. in the steel having the composition defined in the opening paragraph of the specification.

According to my invention and with a view to obtaining in a reliable and uniform manner good and homogeneous steel of the composition given hereinabove, I distinguish those additions which are to remain in the steel obtained and which I add to the aluminothermic mixture, from the deoxidizing or reducing agents which are not intended to remain in the steel obtained and which I add once the aluminothermic reaction, i. e. the reaction of  $Fe_3O_4$  with  $Al$ , has begun. These deoxidizing agents may consist of iron alloys having high contents of deoxidizing elements (more than 75% of Mn or Si) or of compound silicides of Mn or Al or of Mn+Al, etc. . . . or of ferro-titanium, of ferro-vanadium, of ferro-boron, with contents of about 10 to 50% of titanium, vanadium or boron.

Thus, the deoxidizing agents act much more energetically and they afford a greatly improved efficiency without disturbing the principal reduc-

ing reaction  $Al + Fe_3O_4$ . As to the additions which are to remain in the final steel and which are added at the beginning of the process to the aluminothermic mixture, they may according to my invention be incorporated under two forms. The part corresponding to the first form may be added after it has been diluted or alloyed in a metal (steel or alloy) under the form of shavings or grains or the like more or less finely divided parts the percentage of which may reach up to about 40% of the weight of the aluminothermic mixture (aluminium+iron oxide). But the totality of the additions cannot generally be incorporated in this manner as they would excessively cool the aluminothermic reaction.

I am also sometimes lead to retain a certain proportion of soft steel scraps as in the ordinary aluminothermic method.

The remainder of the additions may be added under a generally richer, more concentrated or less temperature-reducing form than for the above mentioned diluted additions. The remainder of the carbon may be added as grains, shavings, turnings of cast iron containing about 2 to 4% of carbon and containing as little as possible of manganese and silicon.

The remainder of the nickel may be added as metallic nickel, ferro-nickel, or nickel oxides. The remainder of the chromium, molybdenum, tungsten, may be added as oxides or iron alloys having reduced contents, say less than 70% of the elements chromium molybdenum, tungsten.

I may use also compound iron alloys containing the desired elements combined two by two, three by three etc. . .

I avoid moreover adding to these alloys elements such as manganese, silicon etc. . . which would have to be eliminated as slags after they have acted.

## Example

Supposing a self-hardening weld steel is to be prepared, having the following composition:

$C=0.3$  to about  $0.6\%$ — $Ni=3$  to about  $3.5\%$ — $Cr=0.8$  to  $1.2\%$  or more—  
 $Mn=0.3$  to about  $0.6\%$ — $Si=$ about  $0.5\%$  or less—  
 $Mo=$ about  $0.075\%$  or more— $P=$ as little as possible—  
 $S=$ as little as possible— $Ti=$ about  $0.1\%$  or less.

I will proceed as follows:  
(a) I add to the aluminothermic mixture having substantially the theoretical proportions viz: 23.7%,  $Al+76.3\% Fe_3O_4$ , firstly 10 to about 20% in weight of a mixture of shavings of a steel

60

65

70

75

80

85

90

95

100

105

110

having for instance one of the two following compositions A or B:

- 5 A: C about 0.3 to 0.6%—Ni about 5 to 7%  
Cr about 0 to 2%—Mo 0.25% or less  
Ti 0.25% or less—Mn 0.4%  
Si 0.5% or less—P and S as little as possible.
- 10 B: C about 2 to 4%  
Ni about 15 to 25%  
Cr about 5 to 10%  
Mo about 0.5% or less  
Ti about 0.5% or less  
Si about 0.5% or less  
Mn about 0.4% or less  
15 P and S as little as possible.

20 The amounts of Mn and Si should be adjusted in accordance with the remaining contents subsequently provided by the deoxidizing agents a small portion of the Mn and Si of which passes into the final steel.

25 Secondly I add the complement required for giving the final steel the desired contents, these contents being added under the form of cast iron grains containing about 2 to 4% of C (for the carbon) of ferro-chromium, nickel or ferro-nickel, ferro-carbon-nickel, ferro-nickel-chromium, ferro-carbon-nickel-chromium etc. . . or oxides of chromium or nickel (for the carbon, chromium and nickel) ferro-molybdenum (for the molybdenum), iron etc. . .

30 (b) Finally as soon as the aluminothermic reaction which is very short (5 to 30 seconds) has begun I add small amounts of deoxidizing agents constituted by ferro-manganese having high contents of manganese, ferro-silicon having high contents of silicon or ferro-silico-aluminium etc. . .

35 This example, of course, is given merely as an indication; other examples could be considered without changing the principle of the invention.

40 What I claim is:

45 1. A method for the aluminothermic preparation of a cast self-hardening steel consisting in incorporating in the aluminothermic mixture of aluminium and iron oxide about 10 to 40% of an alloy in a finely divided state containing elements, selected from a group consisting of C, Cr, Ni, Mo, W, Ti, Bo, Va, Cu, which are to remain in the final steel and in adding only when the aluminothermic reaction has begun, substances having high contents of material acting as deoxidizing agents and selected from a group consisting of manganese, silicon, aluminium, boron, vanadium and titanium.

50 2. A method for the aluminothermic preparation of a cast self-hardening steel consisting in incorporating in the aluminothermic mixture of aluminium and iron oxide about 10 to 40% of an alloy in a finely divided state containing elements, selected from a group consisting of C, Cr,

Ni, Mo, W, Ti, Bo, Va, Cu, which are to remain in the final steel together with a complementary amount of metallic nickel and in adding only when the aluminothermic reaction has begun, substances having high contents of material acting as deoxidizing agents and selected from a group consisting of manganese, silicon, aluminium, boron, vanadium and titanium.

55 3. A method for the aluminothermic preparation of a cast self-hardening steel consisting in incorporating in the aluminothermic mixture of aluminium and iron oxide about 10 to 40% of an alloy in a finely divided state containing elements, selected from a group consisting of C, Cr, Ni, Mo, W, Ti, Bo, Va, Cu, which are to remain in the final steel together with a complementary amount of oxides of elements selected from a group consisting of Ni, Cr, Mo, W, Cu, Va, Ti, Bo and in adding only when the aluminothermic reaction has begun, substances having high contents of material acting as deoxidizing agents and selected from a group consisting of manganese, silicon, aluminium, boron, vanadium and titanium.

60 4. A method for the aluminothermic preparation of a cast self-hardening steel consisting in incorporating in the aluminothermic mixture of aluminium and iron oxide about 10 to 40% of an alloy in a finely divided state containing elements, selected from a group consisting of C, Cr, Ni, Mo, W, Ti, Bo, Va, Cu, which are to remain in the final steel, the contents of which elements is the highest consistent with a good production of this alloy, together with a complementary alloy containing up to about 4% of carbon and certain elements selected from the above disclosed group, the contents of at least one of said elements being higher than in the preceding alloy without being higher than 70% and in adding only when the aluminothermic reaction has begun, substances having high contents of material acting as deoxidizing agents and selected from a group consisting of manganese, silicon, aluminium, boron, vanadium and titanium.

65 5. A method for the aluminothermic preparation of a cast self-hardening steel consisting in incorporating in the aluminothermic mixture of aluminium and iron oxide about 10 to 40% of an alloy in a finely divided state containing elements, selected from a group consisting of C, Cr, Ni, Mo, W, Ti, Bo, Va, Cu, which are to remain in the final steel together with a complementary amount of cast iron containing up to about 4% of carbon and in adding only when the aluminothermic reaction has begun, substances having high contents of material acting as deoxidizing agents and selected from a group consisting of manganese, silicon, aluminium, boron, vanadium and titanium.

70 CLARENCE LEON DELACHAUX.

135